

# United States Patent [19]

Hagita et al.

[11] Patent Number: 4,688,411

[45] Date of Patent: Aug. 25, 1987

[54] **METHOD FOR CONTINUOUS DRAWING OF WIRE ROD**

[75] Inventors: **Hyoji Hagita; Takashi Fukuda, both of Kitakyushu; Shigeru Maeda, Handa; Hideo Imamura, Handa; Kazutoshi Ogata, Handa; Masahiro Fukuoka, Aichi, all of Japan**

[73] Assignee: **Sumitomo Metal Industries, Inc., Osaka, Japan**

[21] Appl. No.: **942,847**

[22] Filed: **Dec. 17, 1986**

### Related U.S. Application Data

[63] Continuation of Ser. No. 733,794, May 14, 1985, abandoned.

[51] Int. Cl.<sup>4</sup> ..... **B21C 9/02**

[52] U.S. Cl. ..... **72/42**

[58] Field of Search ..... **72/39, 41, 42, 43, 44, 72/46, 274; 148/6.15 R, 6.15 Z; 427/318, 327; 252/12**

[56] **References Cited**

### U.S. PATENT DOCUMENTS

2,871,140 1/1959 Goss ..... 72/42 X  
2,990,610 7/1961 Luckerath et al. ..... 72/42  
3,250,103 5/1966 Beaubien et al. ..... 72/42  
3,923,673 12/1975 Van Henten et al. ..... 72/42  
4,308,182 12/1981 Eckard et al. ..... 72/42 X

4,529,451 7/1985 Otrhalek et al. ..... 148/6.15 Z  
4,553,416 11/1985 Sudoh et al. ..... 72/40  
4,575,430 3/1986 Periard et al. ..... 72/42 X

### FOREIGN PATENT DOCUMENTS

0053636 6/1982 European Pat. Off. .  
1103108 3/1961 Fed. Rep. of Germany .  
2402702 8/1974 Fed. Rep. of Germany .... 148/6.15 Z  
2357045 5/1975 Fed. Rep. of Germany .  
204420 11/1983 German Democratic Rep. .

Primary Examiner—E. Michael Combs

Attorney, Agent, or Firm—Burns, Doane, Swecker & Mathis

[57]

### ABSTRACT

A wire rod is payed out from a pay-off stand and descaled in a descaling process. After preheating to a predetermined temperature by a preheating device, it is subjected to a lubrication pretreatment through a zinc calcium phosphate solution applied with ultrasonic wave in the lubrication pretreatment process. After rinsing process, the lubrication-pretreated wire rod is coated with a calcium stearate or a sodium stearate in lubricating process. Thereafter, the wire rod is dried sufficiently in drying process, and then added with a predies lubricant in wire drawing process and coiled by a coiler.

7 Claims, 14 Drawing Figures



FIG. 1



FIG. 2



FIG. 3



FIG. 4



FIG. 5



FIG. 6



FIG. 7



FIG. 8



FIG. 9



FIG. 10



FIG. 11(a) FIG. 11(b)



FIG. 12



FIG. 13



**METHOD FOR CONTINUOUS DRAWING OF  
WIRE ROD**

This application is a continuation of application Ser. No. 733,794, filed May 14, 1985 abandoned.

The present invention relates to a method for continuous drawing of a wire rod for cold-forging, in which the wire rod (inclusive of a steel bar) is descaled, pretreated for lubrication, lubricated and drawn into wire while being moved continuously.

Secondary working for a wire rod for cold-forging is performed normally in the order: descaling (pickling)—lubrication—pretreatment—lubrication—drying—wire drawing—coiling. Among them, pickling, lubrication pretreatment and lubrication are usually rendered in batch treatment system. That is, heretofore, a pickled wire rod coil was dipped in a phosphate solution of, for example, zinc phosphate and, thereafter, dipped in a lubricate solution of, for example, sodium stearate to form a lubricate coating of such materials as sodium stearate, zinc stearate, or zinc phosphate on the surface of the wire rod. The batch treatment system was heretofore used for the reason that a long period of reaction was required to obtain a coating having a thickness sufficient to provide satisfactory lubricating properties, this required a longer treatment time and made an in-line system difficult.

Therefore, in, for example, Japanese Patent Public Disclosure No. 163047/1981 Official Gazette, there is proposed a method for performing lubrication pretreatment and lubrication in an in-line system to thereby reduce equipment cost and improve productivity. This prior art method has been put into practical use. This prior art method is characterized in that, after descaling, a wire rod is coated with zinc phosphate (lubrication pretreatment), further coated thereon with calcium stearate at room temperature (lubrication), and then rapidly dried. In this prior art method, it is made possible to reduce running cost, to coat a required quantity of lubricant in a very short time, to dry it in a short time, and to make it in an in-line system without extending the entire line unduly.

According to prior art methods, however, any of the batch treatment system or the in-line system used zinc phosphate solution as the lubrication pretreatment, and therefore, had a disadvantage that the lubricant coating had unsatisfactory resistance to heat.

Generally in metal wire drawing operation, as described above, lubricant is indispensable to improve the working efficiency, to prolong the tool life, and to maintain the surface quality of drawn wire.

The lubricant for wire drawing reduces the friction between the dies and the wire rod to thereby make it possible to draw the wire rod with a smaller drawing force and prevents wear of the dies. In addition to these functions, the lubricant has important advantage that it remains securely as a coating on the surface of the wire after drawing and acts as an effective lubricant during cold forming (for example, bolt making).

Heretofore, a predies lubricant having metallic soap as the main component as follows was normally used in drawing wire:

-continued

| additives: | several % (by weight) |
|------------|-----------------------|
|------------|-----------------------|

In the prior art lubricant for wire drawing having metallic soap as the main component in which the metallic soap displays the basic lubricating properties, stearate or palmitate of alkali earth metals or sodium were normally used. The typical inorganic material used in the prior art wire drawing lubricant is lime which prevents temperature rise in heavy working to thereby prevent adhesion between the wire rod and the dies and to control the softening temperature of the lubricant. The additives used in the prior art were one or more of sulfur, molybdenum disulfide and graphite which were added to prevent adhesion between the wire rod and dies under severe wire drawing conditions and to improve the lubricating properties.

However, while the prior art wire drawing lubricant having metallic soap as the main component had better properties than other wet type lubricants, it was still insufficient in the lubricating properties such as resistance to heat produced in drawing and adhesiveness of the lubricant coating formed, which made the life of the wire drawing dies and the life of the dies for cold-forging subsequent to drawing relatively short.

The drawn wire rods are mostly cold-forged into products. However, it has become a recent trend that the lubricant used in the wire drawing is left adhering onto the surface of the wire brought to the cold-forging process so that the wire can be cold-forged into products without adding any lubricant. Therefore, while much better adhesiveness after wire drawing and higher heat-resistance sufficient to prevent cracking in the adhering lubricant coating after wire drawing have been demanded for the lubricant for wire drawing, no successful lubricant for wire drawing which satisfactorily answer to these demands has been found yet.

**SUMMARY OF THE INVENTION**

An object of the present invention is to provide a method for continuous drawing of wire rod, in which the wire rod is descaled, pretreated for lubrication, lubricated, dried and drawn into wire in an in-line system to thereby make it possible to obtain a lubricant coating highly resistant to heat and to carry out the wire drawing operation efficiently in a shorter period of time than prior art methods.

Another object of the present invention is to provide a lubricant for wire drawing, which is capable of overcoming the above-described problems of the prior art lubricants and has highly desirable properties such as reduction in friction, resistance to heat, and deposition and adherence to the wire rod, to thereby prolong the life of the dies for wire drawing and cold-forging.

The continuous wire drawing method according to the present invention is characterized in that a descaled and preheated wire rod is pretreated for lubrication by passing it through a calcium zinc phosphate solution ( $Ca/Zn=0.3-1.0$ ) maintained in the temperature range  $70^{\circ}C.-90^{\circ}C.$  and added with an ultrasonic wave (frequency: 10-60 KHZ, output: 25 W/liter solution), rinsed, lubricated by causing calcium stearate to adhere to it at room temperature or passing it through a sodium stearate solution maintained in the temperature range  $70^{\circ}C.-90^{\circ}C.$ , dried and then drawn into wire. Further, in said wire drawing operation, the predies lubricant having metallic soap as the main component added with

|                     |                    |
|---------------------|--------------------|
| metallic soap:      | 60-80% (by weight) |
| inorganic material: | 20-40% (by weight) |

1-10 weight % of a thermoplastic resin (for example, Teflon, polyethylene, nylon, acrylic resin, polycarbonate) is used.

We have discovered that in wire drawing operation addition of a thermoplastic resin to the prior art predies lubricant having metallic soap as the main component improves the lubricating properties of the lubricant considerably. That is, by adding 1-10% by weight of a thermoplastic resin to the prior art predies lubricant having metallic soap as the main component, the lubricating properties of the lubricant, such as reduction of friction and resistance to heat, can be greatly improved.

Addition of the thermoplastic resin in less than 1% by weight is insufficient to improve the lubricating properties satisfactorily. On the other hand, addition of it in more than 10% by weight increases the cost unduly and may result in generation of thermally decomposing gases during heat treatment after cold-forging. Particularly when any of fluorine-contained polymers is used, addition of it in a percentage higher than specified above is accompanied by the risk of generation of fluorine gas during heat treatment after cold-forging. Accordingly, great care must be taken in determination of the percentage of addition of the thermoplastic resin.

The term "metallic soap" as used herein is to be understood to mean metallic salts other than alkali salt, of, such as, fatty acid, resin acid and naphthenic acid, inclusive of sodium salt of these acids and their mixtures, preferably of common composition (commonly used as wire drawing lubricant) containing calcium stearate or sodium stearate in 90% or more in weight added with one or more of aluminum stearate, zinc stearate and barium stearate in several percent by weight.

Further, the term "a predies lubricant having metallic soap as the main component" as used herein is to be understood to mean any of lubricants containing said metallic soap in 60% or more by weight, inorganic material (such as lime) in 20% or more by weight, and several percent of additives (one or more of sulfur, molybdenum disulfide and graphite), that is, this term is applicable to any of known wire drawing lubricants.

The term "thermoplastic resin" as used herein is to be understood to apply to any of polyethylene resin, polypropylene resin, fluorine-contained polymers known as Teflon (trademark), polystyrene resin, vinyl acetal resin, polyacrylate resin, polymethacrylate resin, polyvinyl chloride resin, polyvinylidene chloride resin, polyacrylonitrile resin, polyvinylether resin, polyvinylketone resin, polyether resin, polycarbonate resin, thermoplastic polyester resin, polyamide resin, diene resin, polyurethane resin, and silicone resin. These resins are used solely or in combination of two or more kinds of them.

The thermoplastic resin is added preferably in the form of powder of the size approximately of 10-20  $\mu\text{m}$  diameter.

#### BRIEF DESCRIPTION OF THE DRAWINGS

The invention will be better understood from the following description taken in connection with the accompanying drawings in which:

FIG. 1 is a block diagram of the process of the method for continuous drawing of wire rod according to the present invention;

FIG. 2 is a graph showing the effect of application of an ultrasonic wave to lubrication pretreatment in the present invention;

FIG. 3 is a graph showing the relationship between the frequency of the ultrasonic wave and the zinc calcium phosphate coating weight;

FIG. 4 is a graph showing the relationship between Ca/Zn ratio of the calcium zinc phosphate coating and the zinc calcium phosphate coating weight;

FIG. 5 is a graph showing the relationship between the concentration of calcium stearate and the calcium stearate coating weight;

FIG. 6 is a graph showing the relationship between the treating time of the sodium stearate and the zinc stearate coating weight;

FIG. 7 is a schematic side view of an apparatus for ultrasonic pretreatment for lubrication;

FIG. 8 is a schematic front view of a treating bath;

FIG. 9 is a graph showing the relationship between the quantity of ethylene tetrafluoride resin added to the predies lubricant having metallic soap as the main component and the drawing force in the wire drawing operation using the lubricant;

FIG. 10 is a graph showing the adhesiveness of the lubricant coating in the cold-forging process;

FIG. 11a is a schematic view of the shape of the cut wire rod before cold-forging;

FIG. 11b is a schematic view of the shape of the product of the cold-forging;

FIG. 12 is a graph showing comparatively the results of Bowden tests of the materials subjected to wire drawing and cold-forging using the lubricant according

30 to the present invention and the conventional lubricant, respectively; and

FIG. 13 is a graph showing the results of Bowden tests of the material in an example of the present invention.

#### DETAILED DESCRIPTION OF THE PREFERRED EMBODIMENTS

With reference now to the drawings and more particularly to FIG. 1 thereof, there is shown in block diagram treating processes of the method according to the present invention. As shown, a wire bar is payed out from a pay-off stand 1 and descaled in descaling process 2 by, for example, shot blasting. Subsequently, the wire rod is preheated by a preheating device 3 to a predetermined temperature (80° C. or higher) and then pretreated for lubrication in lubrication pretreatment process 4 by passing it through a calcium zinc phosphate solution (Ca/Zn=0.3-1.0) added with an ultrasonic wave. The calcium zinc phosphate solution is preheated to the temperature 70°-90° C. Then, after rinsing process 5, the pretreated wire rod is lubricated by calcium stearate or sodium stearate to adhere thereto in lubricating process 6. Lubrication by calcium stearate is carried out at room temperature. However, sodium stearate is to be preheated to 70°-90° C. for lubrication in process 6. After lubricated, the wire rod is dried sufficiently in its lubricant coating in drying process 7, drawn with a predies lubricant in wire drawing process 8, and coiled by coiler 9.

Method of descaling rod used in descaling process 2 is not limited. Any of pickling, shot blasting and roll bending may be used to descale the rod in process 2. Among the three methods mentioned above, shot blasting is most preferable for the phosphate coating in an in-line system.

The method according to the present invention is characterized in that calcium zinc phosphate (Ca/Zn=0.3-1.0) having a good resistance to heat is

used in process 4 to pretreat the wire rod for lubrication. The temperature of removing crystal water of the calcium zinc phosphate coating is 415° C. while the temperature of removing crystal water of the heretofore used zinc phosphate coating is 280°-290° C. This means that the prior art zinc phosphate coating is removed of its crystal water by the heat (normally up to 300° C.) developed during wire drawing operation to thereby cause cracks in the coating. In contrast to this, since the temperature of removing crystal water of the calcium zinc phosphate coating according to the present invention is, as mentioned above, as high as 415° C., no crack is caused in the coating by the wire drawing operation.

The method according to the present invention is characterized in that an ultrasonic wave is used in treatment to obtain a sufficient zinc calcium phosphate coating weight and to control the coating weight. This is because the calcium zinc phosphate solution is less sensitive to chemical conversion treatment than the zinc phosphate solution and is more difficult to obtain the coating weight. However, as shown in FIG. 2, the zinc calcium phosphate coating weight is increased by application of the ultrasonic wave thereto. The results shown in FIG. 2 were obtained under the treatment conditions: concentration 160 points, temperature 80° C., and frequency of the ultrasonic wave 50 KHZ at 1 KW.

As shown in FIG. 3, the frequency of the ultrasonic wave applied to the solution is preferably in the range 10-60 KHZ because the frequency lower than 10 KHZ presents a problem of noise and, on the other hand, the frequency higher than 60 KHZ is less effective to obtain a sufficient coating weight. Output of the ultrasonic wave is preferably 25 W per liter of the solution.

The Ca/Zn ratio of the calcium zinc phosphate coating is determined to 0.3-1.0 for the reason described below. FIG. 4 shows the relationship between the Ca/Zn ratio of the calcium zinc phosphate coating (concentration of the solution 160 points) and the coating weight. As understood from FIG. 4, when the Ca/Zn ratio is lower than 0.3, effect of addition of Ca is small and the resistance to heat is not sufficient. On the other hand, when the Ca/Zn ratio is higher than 1.0, the sensitivity to chemical conversion treatment is not sufficient and it is difficult to obtain a predetermined coating weights ( $\geq 6 \text{ g/m}^2$ ) and of metallic soap ( $\geq 1 \text{ g/m}^2$ ). Accordingly, the Ca/Zn ratio of the calcium zinc coating is preferably in the range 0.3-1.0.

The predetermined coating weight of the calcium zinc phosphate coating weight of 6  $\text{g/m}^2$  or larger is obtained in a short period of time 10-20 seconds only when the concentration of the calcium zinc phosphate solution is 160 points or higher. On the other hand, the concentration of the solution of 200 points or higher is not economical since the coating weight in proportion to the increase in the concentration is not obtained. Here, the lower limit of the coating weight of the calcium zinc phosphate coating is predetermined to 6  $\text{g/m}^2$ . The prior art zinc phosphate coating having lower resistance to heat requires the coating weight of the lower limit 7-8  $\text{g/m}^2$ . However, since the calcium zinc phosphate coating according to the present invention has a high resistance to heat, the coating weight of it can satisfactorily be as low as 6  $\text{g/m}^2$ .

The apparatus used for ultrasonic pretreatment for lubrication in the method according to the present invention may take the construction in which, as shown in

FIGS. 7 and 8, a plurality of ultrasonic wave applying devices 12 are disposed vertically or horizontally in pairs in parallel or staggered positions on the outer peripheral surface of a cylindrical treating bath 11, 5 return pipes 14 are provided between treating solution receivers 13 projecting from the inlet side and the outlet side, respectively, of the treating bath 11 and a treating solution tank 15 to collect treating solution 19 therethrough, and a pump 16 is provided to supply the treating solution from the treating solution tank 15 to the treating bath 11 through piping 17. By the apparatus constructed as described above, the calcium zinc phosphate solution is subjected to the ultrasonic wave and agitated, and caused to rapidly adhere to the surface of a wire rod 18 by cavitation. Further, it is made possible to control the coating weight of the calcium zinc phosphate solution by using or not using the application of the ultrasonic wave or by changing the frequency or the output of the ultrasonic wave applying device.

The lubrication process is carried out after the lubrication pretreatment process by passing the wire rod either (1) through calcium stearate solution at room temperature or (2) through sodium stearate solution heated to the temperature 70°-90° C.

In lubrication with calcium stearate (1), as will be understood from the relationship between the concentration and the coating weight shown in FIG. 5, the concentration must be 300 g/liter or higher in order to obtain the predetermined coating weight of 5  $\text{g/m}^2$  or higher. While any of wet spraying (coating solution) and dry spraying (coating powder) can be used to cause calcium stearate to adhere to the wire rod, coating by wet spraying is preferred in view of the coating weight of the lubricant and the adhesiveness of the lubricant coating. Treating time of 2-3 seconds is normally required for physical adhesion.

In lubrication with sodium stearate (2), batch treatment system can be used. In this lubrication with sodium stearate, substitution takes place between the calcium zinc phosphate coating formed by lubrication pretreatment and the sodium stearate solution to produce a zinc stearate layer which adheres to the surface of the wire rod. In this lubrication, it is normally required to obtain the coating weight of the substitution product layer of 1  $\text{g/m}^2$  or higher. For this purpose, as seen from the relationship between the treating time with sodium stearate and the zinc stearate coating weight shown in FIG. 6, a period of time of 20 seconds or longer is required.

The lubrication (1) or (2) above may be omitted in the case where a predies lubricant is used during wire drawing process.

In the method according to the present invention, the predies lubricant is added to increase the heat-resistance and lubricating properties. The predies lubricant used in the method according to the present invention is the lubricant having metallic soap as the main component added with a thermoplastic resin such as Teflon, polyethylene, nylon, acrilic resin, and polycarbonate in 1-10% by weight. The thermoplastic resin is added to the metallic soap lubricant to make use of the heat-resistance and the low friction of the thermoplastic resin such, for example, as Teflon. Further, the quantity of addition of the thermoplastic resin is determined to 65 1-10% by weight because addition of it in less than 1% is not sufficient to provide an effect to the drawing force and, on the other hand, while a larger quantity of addition of it provides a larger effect, the upper limit of

the quantity of its addition is determined to 10% considering the cost and the fact that the decomposition gas of, for example, Teflon is fluorine gas.

FIG. 9 shows graphically the relationship between the quantity of addition of ethylene tetrafluoride (trademark "Teflon") to the wire drawing lubricant containing metallic soap as the main component (having the content: calcium stearate 70%, lime 27%, and sulfur 3% by weight) and the drawing force required to draw a steel rod (equivalent to S45C of JIS—Japanese Industrial Standard) into wire. The graph of FIG. 9 shows the results of drawing of said steel rod coated with zinc phosphate as the lubrication pretreatment and having the diameter 5.5 mmφ into wires with two different reduction of area, approximately 20% and approximately 30%, respectively.

It is clear from FIG. 9 that the required drawing force shows the tendency to decrease suddenly when the quantity of addition of the ethylene tetrafluoride containing resin exceeds 1% by weight. This tendency has been confirmed to appear likewise when other thermoplastic resin is added. While the graph of FIG. 9 shows that the thermoplastic resin is added preferably in larger quantity from the view to increase the lubrication, the quantity of its addition is required to be limited to 10% by weight or less in view of the environmental pollution and economy as mentioned hereinabove.

FIG. 10 shows graphically the comparative results of the adhesiveness of the lubricant coating to the rod being worked between the predies lubricant with no resin added and the predies lubricant with a thermoplastic resin added.

The wire drawing lubricant, the thermoplastic resin added and the lubrication pretreatment method used in the tests shown in FIG. 10 were the same as those used in the tests of FIG. 9, and the wire rod used was a boron steel equivalent to 10B22M of AISI. The coating weight was measured in the manner described below.

A boron steel rod of the diameter 22 mmφ coated with zinc phosphate or zinc calcium phosphate (pretreatment for lubrication) was drawn into rod of 19.5 mmφ with the reduction of area of approximately 21.4% using both of the predies lubricant added with no resin and the predies lubricant added with ethylene tetrafluoride containing 3% by weight, and subjected to cold-forging (extruding to make bolts) during which sampling is started to find the rate of residual lubricant on the drawn rod (extruding reduction of area=0) at each extruding reduction of area. That is, the adhesiveness of the lubricant coating is understood as the following ratio:

$$\frac{\text{coating weight after extrusion}}{\text{coating weight to mother material}}$$

The larger the value of the rate of residual lubricant coating is, the better the adhesiveness of the coating is or the more the lubricant remains and, accordingly, the less frequently the seizure occurs during the cold-forging operation. In the cold-forging used in the method according to the present invention, a rod (diameter:  $d_0$ ) shown in FIG. 11a is formed to, as shown in FIG. 11b, a bolt-like shape (diameter of shank:  $d_1$ ) leaving a head undrawn, with the ratio of maximum accumulated reduction of area of approximately 80%. In this case, the ratio of reduction of area is given by the formula:

$$\left[ 1 = \left( \frac{d_1}{d_0} \right)^2 \right] \times 100.$$

It is understood from the results shown in FIG. 10 that the predies lubricant added with ethylene tetrafluoride containing 3% by weight is obviously superior in adhesiveness of the lubricant coating to the lubricant added with no resin. This shows that the addition of the ethylene tetrafluoride increases the heat resistance of the lubricant and prevents its deterioration by heat generated during working.

FIG. 12 shows the results of Bowden tests (using a Bowden tester for rubbing the surface of the test piece by a steel ball to determine the coefficient of friction corresponding to the number of sliding times) using extruded rods obtained by the cold-forging process described above (extrusion reduction of area: approximately 79.5%).

It is understood from FIG. 12 that the rod coated thereon with the predies lubricant added with the ethylene tetrafluoride in 3% by weight has obviously lower coefficient of friction than the rod coated thereon with the predies lubricant added with no such resin and is lower in the rise of the coefficient of friction than it. Therefore, FIG. 12 shows that the predies lubricant added with the thermoplastic resin is superior in lubricating properties and adhesiveness of its coating.

## EXAMPLE

By the equipment having the line construction shown in FIG. 1, using shot blasting for descaling of the wire rod, and including the ultrasonic pretreatment apparatus for lubrication shown in FIGS. 7 and 8, a material of 5.5 mmφ (S45C) was drawn in the following operative conditions into rods of 4.95 mmφ and 4.6 mmφ, respectively:

- Operating Conditions**
- (1) Descaling Condition  
Shot blasting Material: steel balls 0.3 mmφ  
Shot Density: approximately 300 Kg/m<sup>2</sup>
  - (2) Preheating Condition  
Steam Blowing: at temperature of 80° C.
  - (3) Lubrication Pretreatment Condition  
Lubrication Pretreating Agent: calcium zinc phosphate solution (Ca/Zn=0.5)  
Treatment Condition: 160 points (concentration )×80° C. (temperature)×15 sec. (reaction time), ultrasonic wave: 50 KHZ, 1 KW
  - (4) Lubricating Condition
    - (i) When using calcium stearate  
Concentration: 300 g/liter  
Temperature: room temperature  
Time: 3 seconds
    - (ii) When using sodium stearate  
Concentration: 90 g/liter  
Temperature: 80° C.  
Time: 25 seconds
  - (5) Drying Condition  
Infrared Drying Furnace: furnace temperature 80° C.
  - (6) Wire Drawing Condition  
Predies Lubricant: lubricant having calcium stearate as the main component added with Teflon in 3% Reduction of Area:  
approximately 19% (5.5 mmφ→4.59 mmφ)

approximately 30% (5.5 mm $\phi$  → 4.6 mm $\phi$ )  
Wire Drawing Speed: 80 m/mm

Table 1 shows the drawing force in the method according to the present invention in comparison with prior art method (Lubrication Pretreatment: zinc phosphate, Predies Lubrication: only a lubricant on the market having calcium stearate as the main component).

TABLE 1

| Lubricating Condition | Drawing Force                                                                                |          | Ratio of Drawing Reduction of Area (%)<br>5.5 $\phi$ → 4.95 $\phi$<br>(approx. 19%) | 5.5 $\phi$ → 4.6 $\phi$<br>(approx. 30%) |
|-----------------------|----------------------------------------------------------------------------------------------|----------|-------------------------------------------------------------------------------------|------------------------------------------|
|                       |                                                                                              |          |                                                                                     |                                          |
|                       |                                                                                              |          |                                                                                     |                                          |
| Present Invention     |                                                                                              |          |                                                                                     |                                          |
| 1                     | calcium zinc phosphating<br>— predies lubrication<br>added with Teflon                       | 785 Kg.  | 970 Kg                                                                              |                                          |
| 2                     | calcium zinc phosphating<br>— calcium stearate +<br>predies lubrication<br>added with Teflon | 770 Kg   | 950 Kg                                                                              |                                          |
| 3                     | calcium zinc phosphating<br>— sodium stearate +<br>predies lubrication<br>added with Teflon  | 730 Kg   | 910 Kg                                                                              |                                          |
| Prior Art             | zinc phosphating —<br>calcium stearate predies<br>lubrication                                | 822.5 Kg | 1032.5 Kg.                                                                          |                                          |

FIG. 10 shows the results of Bowden tests (lubricating properties and adhesiveness of the lubricant coating) of the rod after winding. Table 2 shows the number of sliding times when  $\mu=0.2$  in comparison between the method according to the present invention and the prior art method.

TABLE 2

|                   | Bowden Sliding Times ( $\mu=0.2$ ) |                         |     |
|-------------------|------------------------------------|-------------------------|-----|
|                   | Ratio of Reduction of Area         |                         |     |
|                   | 5.5 $\phi$ → 4.95 $\phi$           | 5.5 $\phi$ → 4.6 $\phi$ |     |
| Present Invention | 1                                  | 300                     | 215 |
|                   | 2                                  | 330                     | 240 |
|                   | 3                                  | 365                     | 270 |
| Prior Art         |                                    | 92                      | 74  |

Table 3 shows the life of each of the wire drawing dies and the cold-forging dies used for drawing rods under the conditions described above (provided, the drawing reduction of area: 5.5 $\phi$  → 4.95 $\phi$ ) and then cold-forging them into high tension bolt in comparison with such life in the prior art.

TABLE 3

|                   | Life of Wire Drawing and Cold-Forging Dies |                   |
|-------------------|--------------------------------------------|-------------------|
|                   | Wire Drawing Dies                          | Cold-Forging Dies |
| Present Invention | 50 tons                                    | 800 tons          |
| Prior Art         | 10 tons                                    | 240 tons          |

Life is expressed by tons of products before replacement of the dies for wear or damage thereof.

As will be seen from Tables 1 and 2 and FIG. 13, the lubricant coating according to the present invention is superior in heat resistance and adhesiveness to the zinc phosphate coating according to the prior art. Accordingly, the life of the drawing and the cold forging dies is considerably prolonged in the method according to the present invention.

In the method according to the present invention, as described hereinabove, since calcium zinc phosphate is used as the lubrication pretreating agent, it is made possible to obtain a coating having a higher temperature of removing crystal water and a higher heat resistance than the zinc phosphate coating according to the prior art, and since an ultrasonic wave applying device is used, it is made possible to secure and control freely coating weight of the calcium zinc phosphate coating.

- 5 10 Further, since the lubricant pretreated rod is lubricated by calcium stearate or sodium stearate, the lubricating properties as well as the heat resistance can be improved. Moreover, since a prior art lubricant having metallic soap as the main component added with a thermoplastic resin such as Teflon is used as the predies lubricant during wire drawing operation, it is made possible to improve the heat resistance and the lubricating properties of the lubricant coating and to prolong considerably the life of the cold-working tools.
- 15 20 While we have described and illustrated a present preferred method of practicing the invention, it is to be distinctly understood that the invention is not limited thereto but may be otherwise variously practiced within the scope of the following claims.

- 25 30 35 What is claimed is:
1. A method for continuously drawing a wire rod into a wire, comprising the steps of:  
descaling the wire rod;  
preheating the descaled wire rod;  
pretreating the preheated wire rod for lubrication by passing said rod through a calcium zinc phosphate solution heated to 70°-90° C. and having the ratio (Ca/Zn)=0.3-1.0;  
rinsing the pretreated wire rod;  
lubricating the rinsed wire rod by coating said rod with a calcium stearate or a sodium stearate;  
drying the lubricated wire rod;  
lubricating the dried wire by coating said wire with a predies lubricant having metallic soap as the main component added with an ethylene tetrafluoride in 1-10% by weight; and  
drawing the dried wire rod into a wire.

- 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 83

UNITED STATES PATENT AND TRADEMARK OFFICE  
CERTIFICATE OF CORRECTION

PATENT NO. : 4,688,411

DATED : August 25, 1987

INVENTOR(S) : Hyojoji Hagita, et al

It is certified that error appears in the above-identified patent and that said Letters Patent is hereby corrected as shown below:

On the title page assignee should read

[73] Assignee: Sumitomo Metal Industries, Ltd.

[30] Foreign Application Priority Data:

Japan 59-102339 - 5/21/84

Japan 59-164150 - 8/3/84

Signed and Sealed this

Sixteenth Day of February, 1988

*Attest:*

DONALD J. QUIGG

*Attesting Officer*

*Commissioner of Patents and Trademarks*